

## UNITED STATES PATENT OFFICE

2,230,848

PROGRESSIVE BURNING SMOKELESS  
POWDER

Walter P. Regestein, Wilmington, Del., assignor  
to E. I. du Pont de Nemours & Company, Wil-  
mington, Del., a corporation of Delaware

No Drawing. Application October 4, 1939,  
Serial No. 297,868

9 Claims. (Cl. 52—22)

This invention pertains to progressive burning smokeless powder and more particularly to an improved method of producing such powders having high potential strength.

Those engaged in the manufacture of smokeless powders realize that variations in the relative burning rate at different instants during combustion of the powder are accomplished by variations in the ballistic performance of said powder. Consequently, in some cases regulation of the relative burning rates at different instants during combustion has been effected in order that the optimum ballistic performance might be attained. This regulation has led to the development of a class of powders which are commonly referred to as progressive-burning powders.

Although progressive burning powders have been produced by various methods, perhaps the most practicable has been the one whereby the surface of the powder grain is modified by coating with a surface moderator such as diethyl diphenyl urea, dimethyl diphenyl urea, dinitrotoluene, dibutyl phthalate, diethyl phthalate, and the like. These moderators cause the outer layers of the powder to burn more slowly, with the result that the ratio of the pressure development in the later stages of combustion to that at the stages immediately following ignition is materially higher than it would be were the powder not subjected to this coating treatment.

Whereas various methods have been developed which are practicable for coating powders free from explosive liquid nitric esters, such as nitroglycerin for example, none of the methods presently known is completely satisfactory when employed in conjunction with powder grains containing nitroglycerin or its equivalents. The difficulties encountered in the attempt to coat said nitroglycerin-containing smokeless powder arise because of the fact that the coating agent almost invariably must be applied in a liquid or molten state. In order to reduce the coating agent to this condition, it is necessary to employ a solvent for the coating agent or to supply heat sufficient to melt said coating agent, or possibly to use a procedure involving both elevated temperatures and a solvent. The use of elevated temperatures in conjunction with materials containing nitroglycerin not only is generally unsatisfactory because of the hazard involved, but, in addition, such use causes loss of some of the nitroglycerin by volatilization with the result that it is difficult to produce various lots of powder having the same ballistic performance. Like-

wise, if a material which is a solvent for the coating agent be employed, this material almost invariably is also a solvent for the nitroglycerin, so that obvious difficulties again arise.

The object of the present invention is an improved progressive burning nitroglycerin-containing powder. Another object is a novel method for producing such powder, said method being characterized by enhanced safety and ease of operation. A further object is a novel method of adding nitroglycerin to smokeless powder grains. Other objects will become apparent as the invention is described hereinafter.

These objects are attained by treating smokeless powder of predetermined granulation with a coating agent according to known procedure and then adding nitroglycerin or other explosive liquid nitric ester to the coated powder grains, said grains being suspended in a liquid medium at the time the nitroglycerin is brought in contact therewith. Quite unexpectedly, such procedure does not cause substantial change in the effect of the coating agent, that is to say, the ballistic performances of the powders made in accordance with this method are similar to those yielded by powders of the same composition produced by a process wherein the surface moderator is applied to a powder already containing the explosive liquid nitric ester. Moreover, the presence of moderators or coating agents, such as dinitrotoluene, on the surface of the powder grains increases materially the rate at which the powder absorbs the liquid nitric ester.

The process is applicable to granulated smokeless powder compositions generally. These grains may or may not contain a substantial amount of the volatile solvent used for their manufacture. Nor need the grains be made in accordance with any particular process, but instead may be produced by a method involving the colloiding of the nitrocellulose in the presence of water or solutions by the addition of suitable solvents thereto while agitating such mixtures, or the powder grains may be formed by the extrusion of colloided or partially colloided nitrocellulose from a press, in the form of tubes, rods, or the like. Thus, the particular process by which the base grain is made does not constitute a determining factor. However, it may be stated that I find the present process particularly attractive when used in conjunction with a cellular type grain which is produced in accordance with my copending application Serial No. 244,347, filed December 7, 1938, because of the high absorptive capacity of this type

of grain. Likewise, the composition of the powder or base grain, as I prefer to call it, may be varied widely without causing deleterious effects. Thus, the nitrocellulose present in the base grain 5 may be of the soluble type or may be a mixture of soluble and insoluble nitrocellulose.

The base grains are surface treated with a well-known moderator for smokeless powder. Such moderators include dinitrotoluene, either liquid 10 or solid, diethyl diphenyl urea, dimethyl diphenyl urea, dibutyl phthalate, diethyl phthalate, and the like. Although both liquids and solids are included in the foregoing examples, all have the power of gelatinizing or plasticizing nitrocellulose to some extent.

As stated hereinbefore, the coating of the base grain may be effected according to known procedures. Following the coating operation, the 20 surface treated grains are agitated in the presence of water, and the required amount of nitroglycerine is added to the powder-water slurry at the maximum permissible rate. If the rate of addition of the nitroglycerine is materially greater than the rate at which the nitroglycerine 25 is absorbed by the nitrocellulose, agglomeration or caking of the grains of the finished powder will occur. Said maximum rate, of course, is not a constant, but rather must be established for each 30 type of base grain employed. In general, however, said rate decreases as the density of the base grain increases.

The following examples illustrate my novel 35 method in greater detail. They serve merely as specific embodiments and are not intended to limit the invention:

*Example 1*

Twenty-five pounds of a shotgun type powder having a nitrogen content of 12.60% and sieved 40 through a 14-mesh standard screen and caught on a 38-mesh standard screen were coated with five parts of dinitrotoluene by intermingling the powder and coating agent at a temperature of about 75° C. in the presence of water. After 45 coating, the powder, together with 75 lbs. of water, was charged into a vessel provided with means for agitating vigorously the powder-water mixture, the temperature of said mixture was raised to 35° C., and then 10.73 lbs. of nitroglycerin 50 were added to the agitated slurry. Two hours were required for the addition of this quantity of nitroglycerin, the rate of addition decreasing progressively during this time interval. After the addition of the nitroglycerin had been 55 completed, agitation of the mixture was continued for a period of one hour, the temperature being maintained at 40° C. throughout the entire three-hour period. The impregnated powder was separated from the water and then dried. Analysis 60 of the finished powder showed that it contained 30 parts by weight of nitroglycerin. Inspection of the grains failed to reveal the presence of any free nitroglycerin on the surface thereof, nor was there in evidence any undesirable aggregation or clusters of said grains.

*Example 2*

An additional 25 lbs. of the identical base grain described in the foregoing example were treated 70 in the present example. In this instance, however, the base grain was not coated, but instead was charged into the apparatus employed for the addition of nitroglycerin to the powder grains. The method of introducing the nitroglycerin 75 to the powder grain, the ratio of the various in-

gredients, the temperature, etc., were identical with those prevailing in Example 1, so that the resultant powder not only had the same amount of nitroglycerine present, but also had been made in the same manner as the powder described in 5 said example. Inspection of the powder in this case, however, showed that there was a definite tendency for the grains to cling to each other and thus cause the formation of clusters or aggregates, which could not be broken down very 10 readily. Said formation of aggregates indicates that the nitroglycerin was absorbed slowly and thus permitted sufficient nitroglycerin to remain near or on the surface of the powder grain to render said surface soft and sticky. Hence, 15 when two or more grains having such surfaces, came into contact with one another during the course of the operation, they united and became cemented together when the powder was dried.

As stated hereinbefore, explosive liquid nitric 20 esters other than nitroglycerin may be employed quite satisfactorily. Among these may be mentioned tetrinitrolycerin, ethylene glycol dinitrate, trimethylene glycol dinitrate, propylene glycoldinitrate, and the like. When one of these 25 explosive liquid nitric esters is used instead of nitroglycerin, slight modifications in the mode of procedure are made in order to compensate for the differences in the physical properties of the various materials. Thus, for example, if the particular material employed possesses a high solubility in water or a high vapor pressure as compared to nitroglycerin, these factors must be considered in order to produce a finished powder of given composition. The principle of operation, 30 however, remains unchanged.

The desirability of smokeless powders made in accordance with my novel process is indicated by reference to the following example which sets forth the median ballistic performance of various 40 powders adapted for use as .22 calibre long rifle ammunition, said performance representing the results obtained after the firing of many rounds:

*Example 3*

| Powder | Weight of charge, grains | Mean velocity, F. S. | Pressure, lbs./sq.in. | 45 |
|--------|--------------------------|----------------------|-----------------------|----|
| A      | 2.25                     | 1,295                | 21,860                | 50 |
| X      | 2.05                     | 1,312                | 22,710                |    |

In the foregoing example, A represents a coated nitrocellulose-nitroglycerin powder made by a process whereby the nitroglycerin is incorporated before the powder is granulated, the surface moderator being applied after granulation. X represents a cellular type powder coated with 55 3½ parts of diethyl diphenyl urea, produced in accordance with the process described herein. 60

Examination of the velocity and pressure results shows that the ballistic performance of the two powders is substantially equivalent. However, it may be seen that when composition A is employed in order to attain the desired result, 65 it is necessary to use 0.2 gr. or 10% more powder than when X powder is used, so that the advantages of this latter composition are appreciable.

It will be understood that I do not contend that powders made in accordance with the present 70 invention yield ballistic results heretofore unknown. Such is not the case, but all other known methods of producing a powder capable of similar performance entail the disadvantages set forth hereinbefore.

It will be apparent to those skilled in the art that the description herein permits of many variations without departing from the spirit and scope of the invention. Thus, the liquid constituting the medium in which the powder is suspended while the liquid nitric ester is added thereto, may be composed of flash inhibiting salts in aqueous solution. Likewise, the powder at the time of the nitric ester addition may contain varying quantities of solvents, both of the volatile and non-volatile type. Indeed, experiments have shown that in the case of a densely colloided powder, the presence of a quantity of volatile solvent exceeding that usually deemed permissible in a finished powder, is a material aid to the absorption of the liquid nitric ester. I intend therefore to be limited only by the following claims.

I claim:

1. A method of producing a progressive burning smokeless powder of high potential energy, which comprises forming a nitrocellulose base grain, coating said base grain with a moderant and then adding an explosive liquid nitric ester to the coated grain while maintaining said coated grain in a water-suspension.

2. A method of producing a progressive burning smokeless powder of high potential energy, which comprises forming a nitrocellulose base grain, coating said base grain with a moderant that is a plasticizer for nitrocellulose, suspending said coated grain in an aqueous liquid and adding an explosive liquid nitric ester.

3. A method of producing a progressive burning smokeless powder of high potential energy, which comprises coating nitrocellulose base grains with a plasticizer for nitrocellulose, suspending said coated grains in an aqueous liquid, adding an explosive liquid nitric ester to said suspension, separating the resultant powder grains from the liquid and drying said powder.

4. A method of producing a progressive burning smokeless powder, which comprises coating nitrocellulose base grains with a plasticizer for nitrocellulose, agitating said coated grains in the presence of at least an equal quantity of an aqueous liquid, adding nitroglycerin at a rate not exceeding that at which the nitroglycerin is absorbed, separating the resultant powder and drying it.

5. The method of claim 4, wherein the plasticizer for nitrocellulose is dinitrotoluene.

6. The method of claim 4, wherein the plasticizer for nitrocellulose is diethyl-diphenyl-urea.

7. The method of claim 4, wherein the plasticizer for nitrocellulose is dibutyl phthalate.

8. A method of producing a progressive burning smokeless powder, which comprises forming base grains of nitrocellulose structure, coating the surface of said base grains with dinitrotoluene, producing a powder-water suspension by agitating said coated base grains in the presence of about three times their weight of water, adding from 5 to 40 parts by weight of nitroglycerin at a rate substantially equal to that at which the powder absorbs the nitroglycerin, continuing the agitation after all the nitroglycerin has been added, and separating the resultant powder and drying the same.

9. A method of producing a progressive burning smokeless powder of high potential energy, which comprises adding a finely-divided water-soluble solid to the nitrocellulose-containing colloid, extruding said colloid through dies, and cutting it into grains, leaching the grains in water in order to remove the water-soluble solid therefrom, coating the resultant grains with a moderant, suspending said coated grains in an aqueous liquid, and adding an explosive liquid nitric ester to the coated grains while maintaining said coated grains in a water suspension.

WALTER P. REGESTEIN.